

# United States Patent Office

2,763,617

Patented Sept. 18, 1956

1

2,763,617

## LUBRICATING OIL CONTAINING DICYCLOPENTADIENYL IRON AND A WEAR INHIBITING AGENT

Lawrence B. Scott, Lafayette, Alan C. Nixon, Berkeley, and Douglas G. Roddick, Lafayette, Calif., assignors to Shell Development Company, New York, N. Y., a corporation of Delaware

No Drawing. Application October 29, 1953,  
Serial No. 389,162

16 Claims. (Cl. 252—49.7)

This invention relates to lubricants for use in knock-inducing engines, such as spark-ignition internal combustion engines. More particularly, this invention pertains to lubricating compositions possessing knock-reducing and anti-wear properties.

In many instances it has been found desirable to add an anti-knock agent to a lubricant to act in an auxiliary capacity with a knock-inhibited fuel such as fuels containing tetraethyl lead with or without tricresylphosphate, triphenylphosphate, tributylphosphate, in order to economically and effectively increase octane requirement or aid in overcoming the maldistribution problem generally encountered in multi-cylinder engines.

Although ferrocene (dicyclopentadienyl iron) and ferrocene compounds, when added in minor amounts to lubricating oils, effectively act in the manner described above and in addition, often impart a carry-over anti-knock effect in cases where ordinary fuels are used later, however, ferrocene compounds have the disadvantage of causing wear.

It has been found that lubricating compositions of this invention which contain minor, but knock-inhibiting, amounts of a ferrocene compound can be effectively inhibited against wear by addition thereto of a minor amount, generally less than about 5% by weight of a partial or full organic ester of an inorganic acid such as mono-, di- and trihydrocarbyl phosphite, phosphate, phosphinate, phosphonate, arsenite, arsenate, borate, boronate, including the thio analogues, and mixtures thereof and wherein the hydrocarbyl radicals can be the same or different and includes alkyl, aralkyl, alkaryl, aryl, cycloalkyl, and the like.

Ferrocene,  $Fe(C_5H_5)_2$ , also known as dicyclopentadienyl iron, and the preparation thereof, have been described by T. J. Kealy and T. L. Pauson, *Nature*, vol. 168 (1951), p. 1040. Also, R. B. Woodward et al., *J. A. C. S.*, vol. 74 (1952), p. 3458, have described the preparation of various derivatives of ferrocene. Other ferrocene compounds include substituted ferrocenes such as acylated, carboxylated, halogenated, alkylated, aminated and alcoholated ferrocenes, and the like. Thus, diacetylferrocene, ferrocene dicarboxylic acid, bis-( $\beta$ -chloropropionyl) ferrocene, diacryloylferrocene, dichloroferrocene, tetrachloroferrocene, diaminoferroocene, dihydroxyferrocene, diethoxyferrocene, dimethylferrocene, diethylferrocene, tetraethylferrocene, diisopropylferrocene, di-n-propylferrocene, di-n-butylferrocene, diisobutylferrocene, di-octylferrocene, monopropyl monobutyl ferrocene, and other substituted ferrocenes are excellent anti-knock agents, when utilized in lubricating oils.

The second essential additive in composition of this invention is a partial or full organic ester of an inorganic acidic compound of phosphorus, arsenic, boron, titanium, silica and the like. More specifically, the anti-wear agents include partial and full esters of mono-, di- and tri-hydrocarbyl phosphites, phosphates, phosphinates, phosphonites, phosphonates, phosphines; arsenites, arsen-

2

ates, arsines; stibines; borates, boronates; silicates; titanates; including the thio analogues and mixtures thereof and wherein the hydrocarbyl radicals can be alkyl, aralkyl, alkaryl, aryl, cycloalkyl radicals which radicals can contain substituent groups such as halogens, carboxyl, amino, thioether, ether groups, and the like.

Suitable phosphorus or arsenic containing organic acids of acids of phosphorus, such as ortho-pyro-metaphosphoric and phosphorus or hypophosphorus acid; or ar-

senious or arsenic acids include the mono-, di- and trimethyl, ethyl, propyl, butyl, phenyl, cresyl, 4-ethylphenyl, 4-tertiary-butylphenyl, xylenyl, benzyl, phenylethyl, cyclohexyl, trichlorophenyl, 4-chlorobenzylphosphites, phosphates, thiophosphites, thiophosphates, phosphonates, phosphines, arsenites, arsenates, thioarsenites, and thioarsenates. Preferred compounds are tricresyl phosphate, triethylphosphite, tricresyl thiophosphates, dibutyltrichloromethanephosphonate, tricresyl, arsenite, and diethylbenzenearsonate. In the case of silicate and titanates, the tetraalkyl silicates and titanates are preferred.

Esters of boric acid include triethyl, tripropyl, tributyl, tri(methylamyl), tri-n-dodecyl, tri(tetradecyl), tri(2-ethylhexyl), tricresyl, tri(tetrahydrofuryl), tricyclohexyl borates. Also particularly effective are the tri-

alkyl borates and the dialkyl esters of alkylboronic acids in which the alkyl groups attached to oxygen atoms are branched chain alkyl groups, and also the cyclic esters of boric acid or of alkaneboric acid derived from dihydric alcohols.

Typical of the aforementioned trialkyl borates are the trialkyl esters of boric acid and branched chain alcohols, such as diisopropylcarbinol and of methylisobutylcarbinol. Typical of the dialkyl esters of alkaneboronic acids is di(methylisobutylcarbinyl) methaneboronate. Typical cyclic esters of boric acid are the cyclic esters derived from boric acid and 2,4-pentanediol, pinacol, 2,4-dimethylpentane-2,4-diol or 2,4-dimethylhexane-2,4-diol. Also, there may be used the cyclic esters produced by the esterification of methaneboronic acid with diols such as 2,4-pentanediol. Another class of cyclic esters of boric acid which may be employed are:

ethyl 2,4-dimethylhexane-2,4-diol borate, ethyl pentane-2,4-diol borate, ethyl 2,4-dimethyl pentane-2,4-diol borate, ethyl pinacol borate and ethyl 2-methyl pentane-2,4-diol borate.

45 The quantities of each of the anti-knock compounds and anti-wear agents which can be incorporated into the present base compositions such as lubricating oils or fuels will depend somewhat upon the particular anti-knock compound used, the engine in which the material is to be utilized and the degree anti-knock requirement desired to be met. In general, an effective amount of each of said additives for use in lubricating oils can vary from about 0.01% to about 10% and preferably can vary from about 0.1% to about 5% by weight or as low as 0.05% and even 0.01% by weight.

The base oil of this invention in general will be a mineral lubricating oil, but various neutral or synthetic liquid materials having suitable lubricating properties are suitable for use in the compositions of the invention.

60 Thus, the base may be a hydrocarbon oil including the paraffinic, naphthenic types as well as mixtures thereof. The viscosity of these oils may vary over a wide range such as from 45 SUS at 100° F. to 100 SUS at 210° F. The hydrocarbon oils may be blended with fixed oils such as castor oil, lard oil and the like and/or with synthetic lubricants such as polymerized olefins, copolymers of alkylene glycols and alkylene oxides, organic esters, e. g., 2-ethylhexyl sebacate, dioctyl phthalate; polymeric tetrahydrofuran, polyalkyl silicone polymers, e. g., dimethyl silicone polymer and the like. If desired, the synthetic lubricants may be used as the sole base lubricant or as

the predominant base component or admixed with fixed oils and derivatives thereof.

Compositions of this invention are illustrated by the following examples.

*Composition A*

|                         |            |                     |
|-------------------------|------------|---------------------|
| Ferrocene               | percent wt | 0.5                 |
| Tricresylphosphate      | do         | 1.0                 |
| Mineral lubricating oil |            | Essentially balance |

*Composition B*

|                         |            |                     |
|-------------------------|------------|---------------------|
| Dibutyl ferrocene       | percent wt | 4.3                 |
| Tricresylphosphate      | do         | 2.0                 |
| Mineral lubricating oil |            | Essentially balance |

*Composition C*

|                         |            |                     |
|-------------------------|------------|---------------------|
| Dibutylferrocene        | percent wt | 4.3                 |
| Triethylphosphite       | do         | 5.0                 |
| Mineral lubricating oil |            | Essentially balance |

*Composition D*

|                         |            |                     |
|-------------------------|------------|---------------------|
| Ferrocene               | percent wt | 1.0                 |
| Triisopropylborate      | do         | 1.0                 |
| Mineral lubricating oil |            | Essentially balance |

*Composition E*

|                                  |            |                     |
|----------------------------------|------------|---------------------|
| Ferrocene                        | percent wt | 1.2                 |
| Tri(diisopropyl carbonyl) borate | percent wt | 3.0                 |
| Mineral Lubricating oil          |            | Essentially balance |

*Composition F*

|                         |            |                     |
|-------------------------|------------|---------------------|
| Dipropylferrocene       | percent wt | 1.2                 |
| Tricresyl arsenite      | do         | 1.0                 |
| Mineral lubricating oil |            | Essentially balance |

*Composition G*

|                          |            |                     |
|--------------------------|------------|---------------------|
| Ferrocene                | percent wt | 1.5                 |
| Diethyl benzene arsenate | do         | 2.0                 |
| Mineral lubricating oil  |            | Essentially balance |

*Composition H*

|                         |            |                     |
|-------------------------|------------|---------------------|
| Ferrocene               | percent wt | 1.2                 |
| Tricyclohexylphosphate  | do         | 5.0                 |
| Mineral lubricating oil |            | Essentially balance |

*Composition I*

|                         |            |                     |
|-------------------------|------------|---------------------|
| Diethylferrocene        | percent wt | 1.6                 |
| Tricresylphosphate      | do         | 3.0                 |
| Mineral lubricating oil |            | Essentially balance |

*Composition J*

|                          |            |                     |
|--------------------------|------------|---------------------|
| Dipropyl ferrocene       | percent wt | 4.5                 |
| Triisopropyl phosphate   | do         | 4.0                 |
| Di-2-ethylhexyl sebacate |            | Essentially balance |

Compositions A through J showed an octane benefit varying from 2 to 18 octane numbers when tested in the CFR and Lauson engines using a primary fuel and in field tests using both a primary and secondary reference fuel. Compositions A, B, C and D were also tested in CFR and Lauson engines for wear reducing effects and wear was reduced by from 25% to 75% over a base lubricating oil or lubricating oils containing only about 1.2% ferrocene.

Compositions of this invention are particularly effective when used in combination with primary fuels such as fuels containing tetraethyl lead (TEL), iron carbonyl, with or without the added presence of organic phosphates such as tricresylphosphate, triphenylphosphates, triethylphosphites, or various combustion chamber deposit inhibitors, preignition agents, spark plug anti-foulants, anti-oxidants, and the like.

We claim as our invention:

1. A lubricating oil composition comprising a predominant amount of a lubricating oil and a minor but effective knock-reducing amount of a dicyclopentadienyl iron com-

ound containing only iron, carbon and hydrogen in the molecule, and a minor, but effective wear-inhibiting amount of an oil-soluble organic ester of an inorganic acid selected from the group consisting of trihydrocarbyl phosphates, trihydrocarbyl phosphites, trihydrocarbyl arsenates, trihydrocarbyl arsenites and trihydrocarbyl borates.

2. The composition of claim 1 wherein the knock-reducing compound is an alkyl substituted dicyclopentadienyl iron.

3. A lubricating oil composition comprising a predominant amount of a mineral lubricating oil and a minor, but effective, knock-reducing amount of dicyclopentadienyl iron and a minor, but effective, wear-inhibiting amount of an oil-soluble trihydrocarbyl ester of an inorganic acid selected from the group consisting of trihydrocarbyl phosphates, trihydrocarbyl phosphites, trihydrocarbyl arsenates, trihydrocarbyl arsenites and trihydrocarbyl borates.

20 4. A lubricating oil composition comprising a predominant amount of a mineral lubricating oil and a minor, but effective, knock-reducing amount of dicyclopentadienyl iron and a minor, but effective, wear-inhibiting amount of an oil-soluble trihydrocarbyl phosphate.

25 5. A lubricating oil composition comprising a predominant amount of a mineral lubricating oil and a minor, but effective, knock-reducing amount of dicyclopentadienyl iron and a minor, but effective, wear-inhibiting amount of an oil-soluble trihydrocarbyl borate.

30 6. A lubricating oil composition comprising a predominant amount of a mineral lubricating oil and a minor, but effective, knock-reducing amount of dicyclopentadienyl iron and a minor, but effective, wear-inhibiting amount of an oil-soluble trihydrocarbyl arsenate.

35 7. A lubricating oil composition comprising a predominant amount of a mineral lubricating oil and a minor, but effective, knock-reducing amount of dicyclopentadienyl iron and a minor, but effective, wear-inhibiting amount of tricresyl phosphate.

40 8. A lubricating oil composition comprising a predominant amount of a mineral lubricating oil and a minor, but effective, knock-reducing amount of dicyclopentadienyl iron and a minor, but effective, wear-inhibiting amount of triisopropyl borate.

45 9. A lubricating oil composition comprising a predominant amount of a mineral lubricating oil and a minor, but effective, knock-reducing amount of dicyclopentadienyl iron and a minor, but effective, wear-inhibiting amount of tri(diisopropylcarbonyl) borate.

50 10. A lubricating oil composition comprising a predominant amount of a mineral lubricating oil and a minor, but effective, knock-reducing amount of dicyclopentadienyl iron and a minor, but effective, wear-inhibiting amount of tricresyl arsenite.

55 11. A lubricating oil composition comprising a predominant amount of a mineral lubricating oil and a minor, but effective knock-reducing amount of dibutyl dicyclopentadienyl iron and a minor, but effective, wear-inhibiting amount of tricresyl phosphate.

60 12. A lubricating oil composition comprising a predominant amount of a mineral lubricating oil and a minor, but effective knock-reducing amount of dibutyl dicyclopentadienyl iron and a minor, but effective, wear-inhibiting amount of triisopropyl borate.

65 13. A lubricating oil composition comprising a predominant amount of a mineral lubricating oil and a minor, but effective knock-reducing amount of dibutyl dicyclopentadienyl iron and a minor, but effective, wear-inhibiting amount of tri-(disopropylcarbonyl) borate.

70 14. A lubricating oil composition comprising a predominant amount of a mineral lubricating oil and a minor, but effective knock-reducing amount of dibutyl dicyclopentadienyl iron and a minor, but effective, wear-inhibiting amount of tricresyl arsenite.

15. A lubricating oil composition comprising a predominant amount of a mineral lubricating oil and a minor, but effective knock-reducing amount of dibutyl dicyclopentadienyl iron and a minor, but effective, wear-inhibiting amount of tricresyl phosphate.

16. A lubricating oil composition comprising a predominant amount of a mineral lubricating oil and a minor, but effective, knock-reducing amount of diisopropyl dicyclopentadienyl iron and a minor, but effective, wear-inhibiting amount of tricresyl phosphate.

## References Cited in the file of this patent

## UNITED STATES PATENTS

|    |           |               |               |
|----|-----------|---------------|---------------|
| 5  | 2,010,356 | Shappirio     | Aug. 27, 1935 |
|    | 2,053,474 | Graves        | Sept. 8, 1936 |
|    | 2,059,567 | Evans         | Nov. 3, 1936  |
|    | 2,272,133 | Shappirio     | Feb. 3, 1942  |
|    | 2,629,693 | Barton et al. | Feb. 24, 1953 |
| 10 | 2,680,758 | Thomas        | June 8, 1954  |
|    | 2,683,157 | Weinmayer     | July 16, 1954 |